

T. J. FAY.

PROCESS OF TEMPERING METAL.  
APPLICATION FILED NOV. 6, 1913.

1,194,829.

Patented Aug. 15, 1916.



FIGURE 1



FIGURE 2

WITNESSES:

Robert L. Bruck.

Brammar & West.

INVENTOR,

Thomas J. Fay  
By *Will Smith*  
ATTY'S.

# UNITED STATES PATENT OFFICE.

THOMAS J. FAY, OF BROOKLYN, NEW YORK, ASSIGNOR TO THE PERFECTION SPRING COMPANY, OF CLEVELAND, OHIO, A CORPORATION OF OHIO.

## PROCESS OF TEMPERING METAL.

1,194,829.

Specification of Letters Patent. Patented Aug. 15, 1916.

Application filed November 6, 1913. Serial No. 799,480.

To all whom it may concern:

Be it known that I, THOMAS J. FAY, a citizen of the United States, residing at Brooklyn, in the county of Kings and State of New York, have invented a certain new and useful Improvement in Processes of Tempering Metal, of which the following is a full, clear, and exact description, reference being had to the accompanying drawings.

10 This invention relates to a process of tempering steel. While the process and apparatus whereby the process is realized are adapted for tempering other articles, it is contemplated that one of the principal fields 15 of usefulness of the invention will be the tempering of steel plates, such as are used in the manufacture of flat-leaf springs.

One of the objects of this invention is to provide a process of quenching heated steel 20 articles by the use of a series of quenching tanks any one of which may be used, the temperature of the liquid in the several tanks being maintained practically uniform by a circulation which at least in part depends on 25 the rise in temperature produced in any tank by the article immersed therein.

Further objects of the invention will appear hereinafter in connection with the description.

30 In the drawings forming part hereof Figures 1 and 2 represent each a diagrammatic sectional view of a series of liquid-containing tanks, with means for circulating liquid through said tanks and means for cooling 35 such liquid outside of said tanks.

In the said drawing (referring particularly to Fig. 1), A represents a tank for the quenching liquid, which preferably will be oil. This tank is provided with an inlet 40 connection for a conduit B, the inlet connection being located near the bottom and at one end of the tank. C denotes a stand pipe, which extends through the wall of the tank opposite the inlet connection and which is 45 shown as connected with the adjacent wall of a second tank A', above the bottom thereof,—in substantially the same position as the point of connection between the conduit B and the first mentioned tank. A number of 50 tanks, A, A', A<sup>2</sup> and A<sup>3</sup> are shown, all of the said tanks being connected in series, with the stand pipe of one tank discharging through the adjacent wall of the next adjacent tank. The outlet from the last tank in 55 the series communicates with a pump E, the

delivery end of said pump discharging the oil received from said tank into a cooling device F, which is preferably a pressed-steel radiator wherein the heated liquid is spread out into a series of thin disks, the radiator sections being exposed to a cooling liquid in the tank G, which liquid may be circulated through the tank by means of a pump, or in any other well known manner. From the cooler F the oil is delivered through the conduit B to the tank A, in the manner hereinbefore described. When the heated plate is introduced into the tank A, the oil at and near the surface first boils up as the heated metal strikes the same. A high level of the oil is produced, not only by the displacement of the oil by the immersion of the metal thereinto but by the boiling and swelling of the oil under the heat imparted by the plate. This heated oil, at the top of the tank, is removed at once by the skimmer, the plate meanwhile being lowered into the cool current of oil entering through the inlet pipe at the bottom of the tank, which oil flows in a stream along the plate when the latter is at 60 or near the bottom of the tank, thus not only quickly quenching the plate but wiping off any heated oil that might otherwise adhere thereto and preventing any spheroidal action 65 between the oil and the heated plate. By this 70 action, the presence of "spots" in the steel is prevented, and the steel is quickly and uniformly quenched, whereby it is tempered in the most efficient manner. While heated oil is shown as being discharged from the tank 75 A into the tank A' and thence through each succeeding tank in the series, it has been found in practice that economical and efficient results are realized by placing a plurality of tanks in series (say five) and, by circulating a large body of the cooling liquid, 80 realize a very considerable heat-interchange, with a low difference in sensible temperature, so that the presence of several tanks in series 85 does not prevent or impede the realization 90 of a practical result. For instance, if the total difference in sensible temperature is five degrees for five tanks, and five hundred pounds of the quenching liquid is handled 95 and cooled per minute, allowing 0.5 B. T. U. per pound, then fifty B. T. U. of heat will be absorbed per tank, taking the average of the tanks. However, if one tank of the series 100 is taking more steel than another, then, by having, say, five tanks in series, the tank that 105

is being overworked, as it were, is being helped out by the tanks that are not up to maximum work. It will be understood that the several heated articles are immersed in 5 the different tanks respectively, at the same or different times.

In Fig. 2 of the drawing there is shown an arrangement which differs from that shown in Fig. 1 in that the tanks are connected in parallel instead of in series. In Fig. 2, B' denotes a supply conduit having branches B<sup>2</sup>, each of which is connected to the bottom of one side or end of one of the aforesaid tanks. Each branch B<sup>2</sup> may be 10 provided with a valve B<sup>3</sup>, whereby any tank in the set may be put into and out of operation, irrespective of any other tank. Each tank is provided with a stand pipe C', similar to the stand pipe C and similarly located, 15 each stand pipe communicating with a common outlet manifold H, said manifold communicating with the inlet side of the pump E'. This pump is shown as having its discharge side connected with a radiator F', similar to the radiator F, said radiator being located in the tank G' through which the cooling liquid is circulated in the same manner as in the embodiment of the invention shown in Fig. 1. It will be evident 20 that the tank A, shown in Fig. 2, is substantially identical in operation with the tank A of Fig. 1. It will also be evident that each tank in Fig. 2 is more independent of 25 each other tank than is the case with the earlier-described embodiment of the invention; also that the tanks do not so completely aid each other as they do when connected in series.

30 In both systems, however, means are provided whereby the article to be tempered is effectively cooled and whereby the tempera- 35

ture of the quenching liquid is maintained sufficiently uniform through the tanks as to secure substantial uniformity in the tempered product. 45

Having thus described my invention, what I claim is:—

1. The process of tempering which consists in circulating a quenching liquid 50 through a cooler and a connected series of tanks and immersing heated articles in said tanks respectively.

2. The process of tempering which consists in circulating a quenching liquid 55 through a series of tanks each of which has a hot liquid overflow outlet at the top and a cool liquid inlet at the bottom, whereby the temperature of the liquid in the tanks is equalized, and immersing heated articles 60 in said tanks.

3. The process of tempering which consists in circulating a quenching liquid through a cooler and through a succession 65 of tanks arranged in series with an overflow connection from one tank to the lower part of the next in succession, and immersing heated articles in said tanks.

4. The process of maintaining the liquid in a plurality of tempering baths at substantially equal temperature, comprising circulating the liquid through a cooler and through said baths, the circulation in each bath being proportioned to the rise of temperature therein produced by the article 70 being tempered. 75

In testimony whereof, I hereunto affix my signature in the presence of two witnesses.

THOMAS J. FAY.

Witnesses:

BRENNAN B. WEST,  
JOHN G. UTZ.